# EUROPEAN PATENT APPLICATION

(11) **EP 2 045 822 A2**
(43) Date of publication of application: **08.04.2009**
(21) Application number: 08253139.3
(22) Date of filing: 26.09.2008
(51) Int. Cl.: H01F 1/33

(54) **Method of manufacturing a magnetite-coated iron powder**

(30) Priority: 01.10.2007 JP 2007257245
(71) Applicant: TAIYO YUDEN CO., LTD., Taitou-ku Tokyo 110-0005 (JP)
(72) Inventor: Kawano, Kenji, Tokyo 110-0005 (JP); Yogo, Toshinobu, Tokyo 110-0005 (JP)
(74) Representative: Jackson, Richard Eric

(57) **Abstract**

A method of coating magnetite to the surface of an iron powder capable of obtaining an iron powder coated with magnetite with easy control for the film thickness and at a uniform thickness, including a step of putting an iron powder into a reaction liquid containing iron pentacarbonyl and heating the same in an oxidizing atmosphere, or including a step of heating a reaction liquid containing iron pentacarbonyl in a reducing atmosphere thereby precipitating iron particles and a step of heating the reaction liquid in which iron particles are precipitated in an oxidizing atmosphere and coating magnetite to the precipitate iron particles.

## Description

### BACKGROUND OF THE INVENTION

### Field of the Invention

The present invention provides a method of coating magnetite (Fe₃O₄) on the surface of an iron powder which can control the film thickness of magnetite easily.

### Description of the Related Art

In recent years, the operation frequency for circuits forming electronic instruments has been increased to a high frequency region as reaching a GHz level. Therefore, it has been demanded also for electronic parts forming the circuits that they operate normally in a high frequency region. Also for a wire wound type inductor having a magnetic substance core applied with windings, it has been required that the inductor operates normally in the high frequency region. It is necessary that the magnetic substance core used for the wire wound type inductor conforming to high frequency has high saturation magnetization, high magnetic permeability, and high electric resistivity. As the material for forming the magnetic substance core having such electric characteristics, an iron powder coated at the surface with magnetite (Fe₃O₄) is used.

An iron powder coated with magnetite is formed by coating an iron powder particle having high saturation magnetization and high magnetic permeability but low electric resistivity with magnetite having high electric resistivity. As method of forming an iron powder coated with magnetite, there have been proposed a method of heat treating an iron powder thereby oxidizing the surface and a method of bonding an iron powder and an oxide powder by mixing them in a vibrating mill as disclosed in Japanese Unexamined Patent Publication No. 2002-256304.

### SUMMARY OF THE INVENTION

For obtaining a magnetic substance core having high saturation magnetization, high magnetic permeability, and high electric resistivity together, it is necessary to control the film thickness of magnetite coated on the iron powder. That is, in a case where the film thickness of magnetite is larger, while the electric resistivity increases, saturation magnetization and magnetic permeability decrease. On the other hand, in a case where the film thickness of magnetite is small, while saturation magnetization and magnetic permeability increase, the electric resistivity decreases. Accordingly, it is necessary to control the film thickness of magnetite so as to make saturation magnetization, and magnetic permeability, and electric resistivity compatible to each other.

However, in the method of heat treating the iron powder thereby oxidizing the surface, since formation of an oxide film proceeds no more after the oxide film is formed over the entire surface, it is difficult to control the thickness of the oxide film. Further, in the method disclosed in JP-A No. 2002-256304, since the film is formed by a mechanical treatment, the film thickness tends to be varied and control for the thickness of the magnetite is difficult.

The present invention intends to solve the foregoing problem and provide a method capable of obtaining an iron powder which is coated with magnetite with easy control for the film thickness and at a uniform thickness.

The present invention proposes, in a first aspect, a method of manufacturing a magnetite-coated iron powder of coating magnetite on the surface of an iron powder including a step of putting an iron powder in a reaction liquid containing iron pentacarbonyl and heating the same in an oxidizing atmosphere.

When iron pentacarbonyl is heated in the oxidizing atmosphere, a carbonyl ligand is dissociated by pyrolysis and iron as the central metal is oxidized by the oxidizing atmosphere into magnetite and precipitated on the surface of the iron powder in the reaction liquid. In this way, magnetite is precipitated successively to form a film. According to the first aspect of the invention, the magnetite can be formed to a uniform film thickness and the film thickness can be controlled easily.

Further, present invention proposes, in a second aspect, a method of manufacturing a magnetite-coated iron powder including a step of heating a reaction liquid containing iron pentacarbonyl in a reducing atmosphere thereby precipitating iron particles, and a step of heating the reaction liquid in which the iron particles are precipitated in an oxidizing atmosphere thereby coating magnetite on the precipitated iron particles.

The second aspect is identical with the first aspect in that magnetite is formed at a uniform film thickness and the film thickness can be controlled easily but is different from the first aspect in that the iron powder to be coated is formed by pyrolysis of iron pentacarbonyl. Iron pentacarbonyl is pyrolyzed in a reducing atmosphere to precipitate iron particles and then the reaction liquid containing the precipitated iron particles is heated in an oxidizing atmosphere to precipitate magnetite and coat the same on the surface of the previously precipitated iron particles.

According to the second aspect of the invention, since magnetite is coated in a state where the iron particles to be coated is scarcely oxidized, purity of the iron particle is enhanced. Accordingly, the magnetite-coated iron powder by the second aspect of the invention can provide higher permeability and higher saturation magnetization compared with a case of putting the previously prepared iron powder into the reaction liquid. Further, the second aspect of the invention can form the iron particle as a core and provide coating of magnetite to the iron powder continuously.

According to the invention, an iron powder coated with magnetite with easy control for the film thickness and at a uniform thickness can be obtained.

### DESCRIPTION OF THE ACCOMPANYING DRAWINGS

Fig. 1 is a conceptional view showing an apparatus used for the manufacturing method of the invention.

### PREFERRED EMBODIMENTS OF THE INVENTION

A first embodiment according to the manufacturing method of the invention is to be described. Fig. 1 is a conceptional view for an apparatus used in the invention. As shown in Fig. 1, a closed vessel 1 having a heating means 2 and a stirring means 4 is provided. The closed vessel 1 has a solution tank 3 for containing a reaction liquid 5.

At first, the reaction liquid 5 is contained in the solution tank 3. The reaction liquid 5 is a solution containing iron pentacarbonyl. Since iron pentacarbonyl is liquid at a normal temperature, it may be used as it is for the reaction liquid, or it may be mixed with an organic solvent so as to moderate the reaction. The organic solvent to be used herein includes alcohols such as ethanol and 2-methoxy ethanol, and benzene and decaline. The mixing ratio of iron pentacarbonyl and the organic solvent is preferably 1:80 to 1:200 by volume ratio. Since the amount of precipitated magnetite can be controlled by controlling the mixing ratio of iron pentacarbonyl and the organic solvent, the thickness of the magnetite film can be controlled by controlling the mixing ratio of iron pentacarbonyl and the organic solvent.

Successively, an iron powder is placed in the reaction liquid 5. For uniform coating, it is preferred that the iron powder is charged while stirring the reaction liquid 5 by the stirring means 4. The ratio of the iron powder and the reaction liquid 5 is preferably from 1:20 to 1:50 by volume ratio. Successively, after filling an oxidizing atmosphere, the closed vessel 1 is closed tightly. In a case of reaction in the atmosphere, the vessel is closed tightly as it is. The oxidizing atmosphere may also be an atmospheric air. A gas mixed with a nitrogen to lower the oxygen concentration may also be used for moderating the reaction. Further, the stirring means 4 includes, for example, a rotary blade as shown in Fig. 1.

Successively, the oxidizing atmosphere inside the closed vessel 1 is heated by the heating means 2. The reaction liquid 5 is heated by the heated oxidizing atmosphere to pyrolyze iron pentacarbonyl. Since the decomposition temperature of iron pentacarbonyl in a closed system is 150°C, it is heated to a temperature of 150°C or higher. Iron molecules precipitated by pyrolysis of iron pentacarbonyl are oxidized by the oxidizing atmosphere into magnetite. The magnetite is deposited to the surface of the iron powder to form a magnetite film. The thickness of the magnetite film can be controlled depending on the heating temperature and the reaction time. When the magnetite film reaches a desired thickness, the reaction liquid 5 is filtrated to recover an iron powder, which is washed and dried. Thus, the magnetite-coated iron powder is obtained.

Then, a second embodiment according to the manufacturing method of the invention is to be described. The apparatus used herein is as per the conceptional view shown in Fig. 1, which is identical with that for the first embodiment. The second embodiment is different in that the iron powder to be coated is formed by pyrolysis of iron pentacarbonyl.

At first, a reaction liquid 5 is contained in the solution tank 3. The reaction liquid 5 is a solution containing iron pentacarbonyl identical with that for the first embodiment, which may be used as it is as the reaction liquid, or may be mixed with an organic solvent for moderating the reaction. Further, the amount of the iron powder to be precipitated and the particle diameter can be controlled by controlling the mixing ratio of iron pentacarbonyl and the organic solvent. Successively, after filling a reducing atmosphere, the closed vessel 1 is closed tightly. As the reducing atmosphere, a hydrogen gas, a nitrogen-hydrogen mixed gas, etc. may be used.

Successively, the reducing atmosphere inside the closed vessel 1 is heated by the heating means 2. The reaction liquid 5 is heated by the heated reducing atmosphere and iron pentacarbonyl is pyrolyzed while stirring the reaction liquid 5 by the stirring means 4. Since the iron molecules precipitated by pyrolysis of iron pentacarbonyl are in the reducing atmosphere, they are not oxidized but bonded with other iron molecules to form iron particles. The thus obtained iron particle powder is at a high purity. The particle diameter of the iron powder can be controlled depending on the heating temperature and the reaction time.

When the particle diameter of the iron powder reaches a desired size, the closed vessel 1 is opened to replace the reducing atmosphere with an oxidizing atmosphere. The oxidizing atmosphere is identical with that for the first embodiment. Since the concentration of iron pentacarbonyl in the reaction liquid 5 is lowered by the reaction of forming the iron particles, iron pentacarbonyl in an amount to form the magnetite film may be added to the reaction liquid 5 upon replacement of the atmosphere. After completion for the replacement of the atmosphere, the closed vessel 1 is closed tightly.

Successively, the oxidizing atmosphere inside the closed vessel 1 is heated by the heating means 2. The reaction liquid 5 is heated by the heated oxidizing atmosphere and iron pentacarbonyl is pyrolyzed while stirring the reaction liquid 5 by the stirring means 4. The iron molecules precipitated by decomposition of iron pentacarbonyl are oxidized by the oxidizing atmosphere into magnetite in the same manner as in the first embodiment. The magnetite is deposited to the surface of the iron powder to form a magnetite film. When the magnetite film reaches a desired thickness, the reaction liquid 5 is filtered to recover an iron powder, which is cleaned and dried.

Since the magnetite-coated iron powder obtained as described above has a relatively high purity for the iron powder, it has higher magnetic permeability and higher saturation magnetization compared with those obtained by coating magnetite to a previously prepared iron powder.

### [Example]

### (Example 1)

500 mg of iron pentacarbonyl and 5 ml of decaline were mixed to prepare a reaction liquid. Then, a closed vessel of 4.0 cm inner diameter and 19 cm depth having a rotary blade for stirring was provided, and a glass vessel of 3.5 cm inner diameter and 8.0 cm height was placed as a solution tank in the closed vessel. The reaction liquid described above was contained in the solution tank. Then, 320 mg of an iron powder with an average value of the particle diameter of 3 µm was charged in the solution tank while stirring the reaction liquid by the rotary blade. Then, the cover for the closed vessel was closed to seal the vessel.

Then, the closed vessel is heated by a heater wound around the periphery thereof to elevate the temperature in the closed vessel to 350°C. Reaction was carried out at 350°C for 5 hours and, when the temperature was lowered to a room temperature, the reaction liquid was taken out. The taken out reaction liquid was filtered through filter paper (No. 2) and the obtained iron powder was washed with acetone and dried at 150°C for 1 hr.

In addition to the sample (Sample 1) as described above, a sample heated at a reaction temperature of 250°C (Sample 2) and a sample heated at a reaction temperature of 300°C (Sample 3) were provided. The samples were observed by SEM (Scanning Electron Microscope) and XRD (X-Ray Analyzer) to confirm the formation of the magnetite film and measure the film thickness. Further, the samples were filled each in a predetermined amount in a sample case made of an acrylic resin and the saturation magnetization was evaluated at a room temperature by a sample vibration type magnetometer.

The thickness for the magnetite film was 220 nm for Sample 1, 80 nm for Sample 2 and 150 nm for Sample 3. The electric resistivity was 10.52 Ωm for Sample 1, 0.32 Ωm for Sample 2, and 3.58 Ωm for Sample 3. Further, saturation magnetization was 173 emu/g for Sample 1, 216 emu/g for Sample 2, and 209 emu/g for Sample 3. As described above, it has been found that the film thickness can be controlled easily and the electric resistivity and the saturation magnetization can be controlled by controlling the reaction temperature according to the invention.

### (Example 2)

500 mg of iron pentacarbonyl and 5 ml of decaline were mixed to prepare a reaction liquid. Then, a closed vessel of 4.0 cm inner diameter and 19 cm depth having a rotary blade for stirring was provided, and a glass vessel of 3.5 cm inner diameter and 8.0 cm height was placed as a solution tank in the closed vessel. The reaction liquid described above was contained in the solution tank. Then, a nitrogen-hydrogen mixed gas comprising 97% nitrogen and 3% hydrogen was filled inside the closed vessel and the cover is closed to seal the vessel.

Then, the closed vessel was heated by a heater wound around the periphery thereof to elevate the temperature in the closed vessel to 250°C. Reaction was carried out at 250°C for 5 hours while stirring the reaction liquid by the rotary blade to form 93 mg of an iron powder with an average value of 3 µm for the particle diameter.

Then, the cover for the closed vessel was opened to replace the nitrogen-hydrogen mixed gas with an atmospheric air. Then, 150 mg of iron pentacarbonyl was added to the reaction liquid in the solution tank. Then, the cover for the closed vessel was closed to seal the vessel.

Then, the closed vessel was heated by a heater wound around the periphery thereof to elevate the temperature in the closed vessel to 380°C. Reaction was carried out at 380°C for 5 hours and, when the temperature was lowered subsequently to a room temperature, the reaction liquid was taken out. The taken out reaction liquid was filtered through filter paper (No. 2) and the obtained iron powder was washed with acetone and dried at 150°C for 1 hr.

In addition to the sample (Sample 4), a sample with addition of 100 mg of iron pentacarbonyl (Sample 5) and a sample with addition of 200 mg of iron pentacarbonyl (Sample 6) were provided. The samples were observed by SEM (Scanning Electron Microscope) and XRD (X-Ray Analyzer) to confirm the formation of the magnetite film and measure the film thickness. Further, for the samples, electric resistivity and saturation magnetization were measured in the same manner as in Example 1.

The thickness for the magnetite film was 200 nm for Sample 4, 120 nm for Sample 5 and 280 nm for Sample 6. The electric resistivity was 9.72 Ωm for Sample 4, 3.02 Ωm for Sample 5 and 12.5 Ωm for Sample 6. Further, saturation magnetization was 190 emu/g for Sample 4, 200 emu/g for Sample 5, and 162 emu/g for Sample 6. As described above, it was found that the film thickness could be controlled easily and electric resistivity and saturation magnetization can be controlled by controlling the concentration of iron pentacarbonyl according to the invention. When the Sample 1 and Sample 4 were compared, it was found that the Sample 4 has higher saturation magnetization.

The present invention can be used for the manufacture of a magnetic substance material used for a magnetic substance core of a wire wound inductor conforming to high frequency use and it can be used also for a rust-prevention treatment of an iron powder.

## Claims

1. A method of manufacturing a magnetite-coated iron powder of coating magnetite to the surface of an iron powder, including a step of putting an iron powder into a reaction liquid containing iron pentacarbonyl and heating the same in an oxidizing atmosphere.

2. The method of claim 1, wherein the mixing ratio of iron pentacarbonyl and organic solvent is 1:80 to 1:200 by volume ratio.

3. The method of claim 1 or claim 2, wherein the ratio of iron powder and reaction liquid is from 1: 20 to 1: 50 by volume ratio.

4. A method of manufacturing a magnetite-coated iron powder of coating magnetite to the surface of an iron powder, including a step of heating a reaction liquid containing iron pentacarbonyl in a reducing atmosphere thereby precipitating iron particles, and a step of heating the reaction solution in which the iron particles are precipitated in an oxidizing atmosphere thereby coating magnetite to the precipitated iron particles.
